

No. 789,341.

PATENTED MAY 9, 1905.

B. F. TAYLOR.

METHOD OF TREATING COTTON WOOL.

APPLICATION FILED OCT. 28, 1901. RENEWED AUG. 25, 1904.

Fig. 1.



Fig. 2.



Fig. 3.



Fig. 5.



Fig. 4.

WITNESSES:

W. H. Seely.

W. D. Jennings.

INVENTOR  
Benjamin F. Taylor.

BY Geo. W. Phillips

his ATTORNEY

## UNITED STATES PATENT OFFICE.

BENJAMIN F. TAYLOR, OF BRIDGEPORT, CONNECTICUT, ASSIGNOR TO  
CHARLES A. COE, OF BOSTON, MASSACHUSETTS.

## METHOD OF TREATING COTTON-WOOL.

SPECIFICATION forming part of Letters Patent No. 789,341, dated May 9, 1905.

Application filed October 28, 1901. Renewed August 25, 1904. Serial No. 222,347.

To all whom it may concern:

Be it known that I, BENJAMIN F. TAYLOR, a citizen of the United States, and a resident of Bridgeport, in the county of Fairfield and 5 State of Connecticut, have invented a certain new and useful Method of Treating Cotton-Wool, of which the following is a specification.

My invention relates to an improved method 10 of treating raw cotton or the so-called "cotton-wool" so as to give increased tenacity or firmness to the staple; and it consists in coating the fiber or staple of the cotton with carbon deposits, as will hereinafter be more fully set forth in the following specification.

15 To enable others to understand my invention, reference is had to the accompanying drawings, in which—

Figure 1 represents a view of the outer surface of a strip of raw cotton after treatment. 20 Fig. 2 is a view of the surface of a cotton strip before being coated with carbon deposits. Figs. 3 and 4 show the manner of depositing the carbon. Fig. 5 is a cross-sectional view of a bicycle-tire, showing the carbonaceous cotton utilized as a filling material to afford a protection against puncture of the 25 pneumatic tire, which is only one of the uses for which the carbonaceous cotton is adapted.

It is well understood that each individual 30 fiber of cotton is hollow, and such fiber contains more or less of water and vegetable oils. My method consists in exposing the cotton-wool to a degree of heat sufficient to convert the evaporative portions of the oil 35 and water into gases, which passing off will leave a carbon deposit or residue within the fiber and also on the outer surface of the same if water and oil were present thereon.

At Fig. 2 is seen a strip of raw cotton before it is treated. It will be observed that the fiber is inclined to be substantially straight—not straight, however, in the strict sense of the term, as would be the case with fur, but much straighter than woolen fiber. This cotton strip is held over a burning substance 45 that is rich in carbon and at a distance therefrom (see Fig. 3) to be at first only affected by the carbonic-acid gases. The heat will be sufficient to evaporate the moisture and thor-

oughly dry the cotton, and at the same time 50 the carbonic-acid gases will carry sufficient carbon to thinly coat or discolor the cotton fibers. After remaining in this elevated position for a few moments to effect the results just described it is dropped to a lower plane 55 or the burning material is elevated, as the case may be, where the carbon will be deposited more rapidly. The cotton is thus moved from point to point until it can finally occupy a position (see Fig. 4) that is richest in carbon 60 escaping from the point of combustion, and the carbon at this last point will of course deposit more rapidly than at any other point of suspension. It is quite evident that if the cotton in the first instance had been placed at 65 the lowest point, as shown at Fig. 4, it would ignite and burn up before sufficient carbon had deposited to protect the fibers against the high temperature at this low point; but by approaching gradually this point of high 70 temperature the fibers are fully protected before they reach such lower position. This carbon deposit will make the cotton fibers tougher and more tenacious; besides, the heat will cause the several hairy fibers to curl up, 75 as shown at Fig. 1, and this curling of the fibers will then resemble more nearly a high grade of sheep's wool.

It is well known that the fibers of raw cotton or cotton-wool when arranged in sheets offer 80 but little resistance to lateral strains, owing to the fact that the loose straight or comparatively straight fibers do not interlock with each other with the same degree of tenacity as sheep's wool. For that reason it cannot 85 be employed exclusively for felting. Therefore it is customary to mix a certain quantity of high-grade sheep's wool with the raw cotton in order to secure the proper tenacity. The carbonaceous cotton will so increase 90 its tenacious qualities that the sheep's wool can be entirely omitted, thereby reducing the cost of felt without interfering with the grade or quality.

Among the many uses for which the carbonaceous cotton can be employed is as an elastic non-puncturable filler for bicycle-tires, as shown at Fig. 5. 1 represents a section of

a pneumatic tire having the lower air-chamber 2 separated from an upper chamber containing the filling material by means of the flexible diaphragm 3. 4 is the carbonaceous cotton filler placed in this upper chamber. This carbonaceous cotton is arranged in a continuous unbroken sheet and rolled up, as shown, filling said chamber and extending entirely around the tire. This carbonaceous cotton is not only tougher, and thereby harder to puncture, but its resiliency is also increased however it may be placed in the tire—whether rolled, as shown, or deposited in layers.

15 While I show and describe a certain process whereby the cotton fibers are impregnated with carbon, this process may, if desired, be varied in order to secure the same result, for my invention consists, essentially, in subjecting the cotton to heat and carbon deposits thrown off from a burning substance or smudge.

20 As before mentioned, the first step in my improved method is to subject the cotton to a heat sufficient to cause its fibers to curl up or interlock, the carbonization or depositing of carbon being of course a preferably added step.

25 Having thus described my invention, what I claim as new, and desire to secure by Letters Patent, is—

30 1. The method of treating cotton which consists in subjecting the cotton to a dry heat

containing carbon sufficient to cause the fibers to curl and thereby render them more liable 35 to interlock or intermesh with each other, for the purpose set forth.

2. The herein-described method of treating cotton-wool so as to increase its tenacity and resiliency, which consists in exposing the cotton to the direct action of heat and coating the same with carbon deposits emanating from the burning matter which furnishes the heat, for the purpose set forth.

3. The herein-described method for treating 45 cotton-wool so as to increase its tenacity and resiliency which consists in subjecting the cotton-wool to a heat sufficient to expel the moisture and thus leave it richer in carbon both on the interior and exterior of the fibers 50 so as to protect against a higher temperature, then, increasing the temperature and quantity of carbonaceous matter until the fibers are sufficiently coated with carbon deposits, substantially as set forth.

4. The method of treating cotton to heat and carbonaceous matter so as to increase the tenacity of its fibers, for the purpose set forth.

Signed at Bridgeport, in the county of 60  
Fairfield and State of Connecticut, this 25th  
day of September, A. D. 1901.

BENJAMIN F. TAYLOR.

Witnesses:

W. Y. SEELEY,  
A. K. LOVELL.